# EUROPEAN PATENT SPECIFICATION

(11) **EP 3 746 588 B1**
(45) Date of publication and mention of the grant of the patent: **30.07.2025**
(21) Application number: 19748287.0
(22) Date of filing: 31.01.2019
(51) Int. Cl.: D02G 3/04, D02G 3/02, D02G 3/22, D01D 5/253, D01D 5/20, D01D 5/26, D01F 8/14, D01G 1/04, D01G 1/10, A41D 31/12

(54) **MULTI-LENGTH, MULTI-DENIER, MULTI-CROSS SECTION FIBER BLEND YARN**
FASERMISCHUNGSGARN MIT MEHREREN LÄNGEN, MEHREREN DENIER UND MEHREREN QUERSCHNITTEN
FIL DE MÉLANGE DE FIBRES À MULTIPLES LONGUEURS, MULTIPLES DENIERS ET MULTIPLES SECTIONS TRANSVERSALES

(30) Priority: 31.01.2018 US 201862624422 P; 17.10.2018 US 201862746619 P; 30.01.2019 US 201916262234
(43) Date of publication of application: 09.12.2020
(73) Proprietor: Parkdale Incorporated, Gastonia, NC 28054 (US)
(72) Inventor: USHER JR, Robert A., Charlotte, North Carolina 28277 (US)
(74) Representative: Tomkins & Co
(86) International application number: PCT/US2019/015996
(87) International publication number: WO 2019/152615

(56) References cited:
- WO-A1-2007/040848
- JP-A- 2007 247 127
- JP-A- 2012 219 396
- US-A- 3 831 481
- US-A- 3 965 664
- US-A- 4 384 450
- US-A- 4 497 231
- US-A- 4 538 490
- US-A- 4 569 264
- US-A- 4 991 387
- US-A- 5 188 892
- US-B2- 9 663 876

## Description

### Background

The present invention relates to fibers, yarns and fabrics in the arena of technical wear, athletic wear or "athleisure" wear.

The market for specialized garments for athletic and leisurewear has grown remarkably in recent years. This in turn has led to the development of, and the further desire to develop, specialized fabrics for such end uses. As is well understood by the skilled person in textiles, the performance of a garment is based upon the fabric from which it is cut and sewn, with the fabric in turn reflecting the properties of the yarn from which it is woven or knitted, and the properties of the yarn reflecting the staple fibers from which the yarn is formed.

Accordingly, since the development and understanding of polymers beginning in the early 20th century, textile chemists have sought to mimic the best properties of natural fibers (cotton, wool, linen) as well as to tailor fiber properties to specific end uses.

Cotton is an extremely comfortable fiber in many circumstances and cotton garments remain ubiquitous based on their light weight, versatility, and favorable hand. The term "hand" is used throughout this application in the sense that is well understood to the skilled person. It can be defined as, "a characteristic of fabrics that is perceived by touching, squeezing, or rubbing them" (Tortora at page 262), or as, "the "term used to describe the feel of a substrate (i.e., soft, raspy, stiff, etc.)" (Textile Glossary; Cotton Incorporated; www.cottoninc.com; accessed March 15, 2018.

Nevertheless, and with particular respect to athletic or active wear, cotton has certain disadvantages. Cotton is highly absorbent, taking up to 27 times its weight in water, which adds undesired weight in the athletic wear context. Cotton also loses its insulating properties and can be abrasive when wet. Thus, in cold weather, active exercise (or work, etc.) cotton layers next to the skin quickly become wet, heavy, and cold. Cotton undergarments become abrasive when wet in both hot and cold weather.

Wool has excellent insulating properties, can stretch as much as 30% beyond its relaxed length, and can absorb moisture in up to 50% of its dry weight without becoming saturated, Tortora, FAIRCHILD'S DICTIONARY OF TEXTILES, 7th Ed. (2009), page 634. Some types of wool are, however, uncomfortable next to the skin, and the more comfortable fibers (e.g., merino) tend to be more expensive. Silk is, of course, extremely comfortable, but in general too expensive for widespread use in mass-marketed athletic garments.

Accordingly, much effort (and with some success), has been placed into developing synthetic-based fabrics from synthetic fibers, or blends of synthetic fibers with natural fibers; e.g., Dacron and wool, cotton and polyester, etc. Additionally, further effort has been applied to developing fully synthetic garments that mimic the comfortable hand of cotton, while providing better moisture management then standard cotton or common cotton-synthetic blends.

The term moisture management is used to describe the capacity or ability of a fabric to pull or wick moisture (perspiration, humidity, rain) to an outer layer of a fabric from which it can evaporate. In many circumstances body temperature (98.6°F, 37°) can help drive wicking in fabric garments, particularly given that entropy will generally favor the vapor (i.e., more random) state. Moisture management is thus typically measured using water vapor transmission rate.

Synthetics are not an automatic cure-all, however, because overcooling can give a clammy feel to the wearer. Accordingly, modern "technical" wear often consists of two types of yarn formed into several layers that are arranged so that thermodynamics drives perspiration from the skin to the first layer and then from the first layer to the outer layer. Modern technical fabrics may have as many as four or five layers for this purpose.

Furthermore, because the starting fibers help establish the properties of the resulting fabric, the skilled person recognizes that with respect to (for example) cotton, shorter fibers produce yarns that in turn give fabrics with a better hand, while longer fibers give smoother more finished yarns, such as those that give a cotton business shirt (again, as just one example) a more finished look, but a rougher hand.

The spinning technique (ring versus open end) likewise makes a difference in the appearance and hand of a finished garment.

US4384450A discloses a polyester yarn containing six groups of fibers of different lengths.

Accordingly the goal remains of designing specialized yarns that produce desired combinations of hand and moisture management.

### Summary

According to the present invention, there is provided a spun yarn according to claim 1.

In another embodiment the invention is an intimately blended bale of polyester staple fibers according to claim 4.

In another embodiment the invention is a fabric according to claim 5.

Preferably the fabric is selected from the group consisting of woven fabrics, nonwoven fabrics, and knitted fabrics.

In another embodiment the invention is a method of making a yarn precursor blend according to claim 9.

Also disclosed is a method of making a yarn with selected properties of moisture management and hand, that includes the steps of opening an intimately blended bale of staple fibers in at least three different deniers, at least four different lengths, and at least two different cross sections, and forming the opened staple fibers into tow, forming the tow into a roving; and spinning the roving into yarn.

Also disclosed is a method of making yarn that includes comprising opening an intimately blended bale that consists essentially of (1) a combination of polyester staple fibers with staple lengths of 1.5 inches (3.81 cm), 1.25 inches (3.175 cm), 1.0 inch (2.54 cm) and 0.75 inch (1.905 cm); (2) a combination of polyester staple fibers with staple deniers (tex, fineness) of 1.0 dpf (111 mtex), 1.2 dpf (133 mtex) and 1.5 dpf (167 mtex); and (3) a combination of polyester staple fibers with at least two different staple cross sections.
Also disclosed herein is a reel assembly for use with a staple cutting apparatus that includes a cutter reel having a pair of annular reel members spaced axially one from the other with each reel member defining an outwardly facing axial surface having a predetermined diameter and a circumferential mating engagement portion; a plurality of cutter blades mounted in said reel members for engaging and cutting fiber; and a cover member encircling and affixed about one of the reel members; in which the improvement comprising cutter blades spaced to cut synthetic filament into discrete staple lengths of 1.5 inches (3.81 cm), 1.25 inches (3.175 cm), 1.0 inch (2.54 cm) and 0.75 inch (1.905 cm).

The foregoing and other objects and advantages of the invention and the manner in which the same are accomplished will become clearer based on the followed detailed description taken in conjunction with the accompanying drawings.

### Brief Description of the Drawings

Figure 1 is a micrograph of fibers with elliptical (oval) cross-sections according to the present invention.
Figure 2 is a fiber length histogram based on one sample of a yarn according to the present invention.
Figure 3 is a second fiber length histogram based on the same sample as Figure 2.
Figure 4 is a fineness (denier, tex) histogram based on the same sample as Figures 2 and 3.
Figure 5 is a fiber length histogram based on a second sample of a yarn according to the present invention.
Figure 6 is a second fiber length histogram based on the same second sample as Figure 5.
Figure 7 s a fineness (denier, ex) histogram based on the same sample as Figures 5 and 6.
Figure 8 is a combination view of an assembled cutter reel and an exploded cutter reel that can be used to practice aspects of the present invention.

### Detailed Description

As used herein, the term polyester refers to any polymer formed by joining hydrocarbon chains with ester groups (Tortora, page 437). The US Federal Trade Commission defines polyester as, "[A] manufactured fiber in which the fiber-forming substance is any long chain synthetic polymer composed of at least 85% by weight of an ester of a substituted aromatic carboxylic acid, including but not restricted to substituted terephthalate units." 16 C.F.R. § 303.7(c)(2018).

Bale Density: A unit of measurement of weight per unit volume normally expressed as pounds per cubic foot. Density is calculated by dividing the net bale weight by the bale volume in cubic feet. Volume is determined by multiplying bale length, width and thickness dimensions expressed in feet. Thickness is determined by measuring from tie to tie across the crown of the bale.

Universal Density (UD): Cotton bale density of at least 28 pounds per cubic foot.

Standard Density (SD): Cotton bale density of at least 23 pounds per cubic foot but less than 28 pounds per cubic foot.

Gin UD: Bale compressed at the gin to a density of at least 28 pounds per cubic foot.

(Bale must be tied with strapping or wire as defined under Section 1.1 and 1.2).

(Bales must be tied with strapping or wire as defined under Section 1.1 and 1.2).

Gin SD: Bale compressed at the gin to a density of at least 23 pounds per cubic foot but less than 28 pounds per cubic foot.
http://www.cotton.orq/tech/bale/specs/definitions.cfm; accessed February 17, 2018
Glossary from National Cotton Council of America7193 Goodlett Farms Parkway Cordova, TN 38016

### Spinning:

As used in the textile industry, the term "spinning" has two distinct meanings. In a classical meaning dating almost to antiquity, "spinning" refers to the step of twisting fibers together to make yarns. In modern technology this is (typically) carried out using "ring" spinning or "open end" spinning, each of which are Familiar to the person of ordinary skill in the art; e.g. Tortora, Fairchilds Dictionary Of Textiles, 7th Ed. (2009) at pages 473 and 395.

In another sense, the word "spinning" is used to refer to the step of extruding a polymer melt into individual filaments which are then processed further, typically including texturing, cutting into "staple" lengths, and spinning the polymer staple fibers into yarns in the open end or ring spinning sense. Tortora at page 536.

The term "opening" is likewise well understood by the skilled person and generally represents a preliminary step in separating staple fibers taken from a compressed bale into looser tufts and removing (where necessary) heavier impurities. Tortora page 395.

As used herein, the term polyester refers to any polymer formed by joining hydrocarbon chains with ester groups (Tortora at page 437).

In a first aspect, the invention is a yarn consisting essentially of a blend of polyester fibers customized by three parameters: (1) a combination of polyester staple fibers with staple lengths of 1.5 inches (3.81 cm), 1.25 inches (3.175 cm), 1.0 inch (2.54 cm) and 0.75 inch (1.905 cm); (2) a combination of polyester staple fibers with staple deniers (tex, fineness) of 1.0 dpf (111 mtex), 1.2 dpf (133 mtex) and 1.5 dpf (167 mtex); and (3) a combination of polyester staple fibers with at least two different staple cross sections including circular and oval cross sections.

In exemplary embodiments, the yarn consist essentially of a blend of polyester fibers in the amounts of 20% by weight staple length of 1.5 inches (3.81 cm) or greater; 54% by weight staple lengths of 1.25 inches (3.175 cm) or greater; 77% by weight staple lengths of 1 inch (2.54 cm) or greater; and 96% by weight staple lengths of 0.75 inch (1.905 cm) or greater; with all lengths and percentages expressed to 2 significant figures.

In such exemplary embodiments the yarn includes 94% by weight of fibers at least 100 mtex; 87% by weight of fibers of at least 125 mtex; 76% by weight of fibers having at least 150 mtex: and 63% of fibers having at least 175 mtex; with all percentages expressed to 2 significant figures.

Table 1 sets forth exemplary length and dpf blends according to the invention. Table 1 (Figure 1)

| **Fiber Length** | | **% of fibers** | **% of fibers (US Pima)** |
|---|---|---|---|
| 0.75" | | 10 | 15 |
| | 1.00" | 20 | 20 |
| | 1.25" | 30 | 25 |
| | 1.5" | 40 | 40 |
| Avg | | 1.25 | |
| **Dpf** | | **for 30's SIRO 100%** | **For 40's CPRS 60/40** |
| | | | |
| | 1 | 20 | 30 |
| | 1.2 | 60 | 60 |
| | 1.5 | 20 | 10 |
| | Avg | 1.22 | 1.17 |
| | | | |

As used in Table 1, 30's SIRO 100% means a 30 Ne yarn. (English yarn count; 30 x 840 yds = 25,200 yards of this yarn weighs 1 pound). It was spun on a SIRO ring spinning machine, in which 2 roving bobbins draft into 1 spinning bobbin, and this yarn was made of 100% polyester fiber in the indicated proportions.

40's CPRS 60/40 means a 40 Ne yarn (English yarn count; 40 x 840 yds = 33,600 yards of this yarn weighs 1 pound). The CP descriptor means combed cotton, so this sample represents 60% combed cotton blended with 40% polyester according to the invention. The RS designation means that this yarn was spun on a standard ring spinning frame, where 1 roving bobbin feeds 1 spinning position. To set forth an alternative, the nomenclature would use the acronym OE, which stands for open end spinning, also called rotor spinning.

The yarn count numbers above are based on length/weight with the standard of yards/pound of yarn. This is the inverse of the denier system, which is based on weight/length.

The data in Tables 2 and 3 were collected on samples of yarn made according to the invention and tested on an USTER^{®} AFIS PRO 2 fiber process control system (Uster Technologies AG, Sonnenbergstrasse 10, 8610 Uster, Switzerland; www.uster.com; https://www.textilemates.com/siro-spinninq-application; accessed February 24, 2018). The listed values are defined as follows:

Tables 2 and 3; Numerical output of results

Neps (a nep is defined as small knot of entangled fibers commonly regarded as a fault but sometimes introduced as an effect. http://www.textileglossary.com/terms/nep.html; accessed February 25, 2018).

Total nep cnt: Count of all neps in a sample (fiber and seed coat neps).

Total nep mean size: Average size of all neps (fiber and seed coat neps) counted in microns.

Fiber nep cnt: Count of all fiber neps.

Fib nep mean size: Average size of all fiber neps in microns.

SC nep count: Count of all seed coat neps.

SC nep mean size: Average size of all seed coat neps in microns.

### Length

L (w) Average fiber length by weight of all the cotton fibers in the sample.

L (w) CV % Variation of the fiber length around the average is expressed as length variation by weight or CV %. CV is used in its well-understood statistical sense to express the ratio of the standard deviation to the mean.

SFC (w) % Percent of all fibers in a cotton sample that are shorter than 12.7 mm (0.5 in.) by weight.

UQL (w) % Length by which 25 % of all fibers by weight exceed in a cotton sample.

L (n) Average fiber length by number of all cotton fibers in the sample.

Variation of the fiber length around the average is expressed as length variation by number or CV %.

SFC (n) % Percent of all fibers in a cotton sample that are shorter than 12.7 mm (0.5 in.) by number.

5 %L (n) Length of the longer 5 % of all fibers in a cotton sample.

### Trash

Total trash count: Count of all particles (dust and trash particles).

Total trash size: Average size of all particles counted (dust and trash particles).

Dust count: Count of all particles less than 500 microns in size.

Dust mean size: Average size of all dust particles counted.

Trash count: Count of all particles greater than 500 microns in size.

Trash mean size: Average size of all trash particles counted VFM %: Calculation taking both dust and trash content as well as size into account; relates to gravimetric trash measurement methods such as Shirley Analyzer.

Statistics Statistical values: Overall measurement protocol with statistical data in the result.

Columns: Mean (Average), Standard deviation, Coefficient of variation CV %, 99 % confidence range, Min. value, Max. value.

**Table 2 (Figures 2-6**

| NEP | Rep | Total Nep Cnt | | Total Nep Mean Size | | Fiber Nep Cnt | | FibNep Mean Size | SCNep Count | | SCNep Mean Size | | |
|---|---|---|---|---|---|---|---|---|---|---|---|---|---|
| | | [Cnt/g] | | [um] | | [Cnt/g] | | [um] | [Cnt/g] | | [um] | | |
| | 1 | 14 | | 592 | | 14 | | 592 | 0 | | 0 | | |
| | 2 | 11 | | 565 | | 11 | | 565 | 0 | | 0 | | |
| | 3 | 14 | | 550 | | 14 | | 550 | 0 | | 0 | | |
| ⁿ | 3 | | | | | | | | | | | | |
| Mean | | 13 | | 569 | | 13 | | 569 | 0 | | 0 | | |
| Std. Dev. | | 2 | | 21 | | 2 | | 21 | 0 | | 0 | | |
| CV% | | 13.3 | | 3.7 | | 13.3 | | 3.7 | 0.0 | | 0.0 | | |
| Q99% | | 11 | | 120 | | 11 | | 120 | 0 | | 0 | | |
| Min | | 11 | | 550 | | 11 | | 550 | 0 | | 0 | | |
| Max | | 14 | | 592 | | 14 | | 592 | 0 | | 0 | | |
| USP | [2013] | <5 | | | | | | | <5 | | | | |

| | | | | | | | | | | | | | |
|---|---|---|---|---|---|---|---|---|---|---|---|---|---|
| LEN | Rep | L(w) | C L(w) CV% | SFC(w) | UQL(w) | L(n) | CV% L(n) | SFC(n) | 5% L(n) | Fineness | Maturity Ratio | IFC | |
| | | [in] | [%CV] | %<0.5 in | [in] | [in] | [%CV] | %<0.5 in | [in] | [mtex] | [mat1] | [%] | |
| | 1 | 1.20 | 28.0 | 0.8 | 1.40 | 1.10 | 30.2 | 2.4 | 1.58 | 184 | 1.10 | 2.8 | |
| | 2 | 1.19 | 27.3 | 0.7 | 1.39 | 1.10 | 29.4 | 1.9 | 1.56 | 177 | 1.10 | 3.0 | |
| | 3 | 1.21 | 26.2 | 0.7 | 1.40 | 1.11 | 28.8 | 2.0 | 1.55 | 176 | 1.10 | 2.7 | |
| ⁿ | 3 | | | | | | | | | | | 2.8 | |
| Mean | | 1.20 | 27.2 | 0.7 | 1.40 | 1.10 | 29.4 | 2.1 | 1.56 | 179 | 1.10 | | |
| Std. Dev. | | 0.01 | 0.9 | 0.1 | 0.00 | 0.01 | 0.8 | 0.2 | 0.02 | 4 | 0.00 | 0.1 | |
| CV% | | 0.6 | 3.3 | 11.9 | 0.3 | 0.9 | 2.7 | 10.7 | 1.1 | 2.4 | 0.4 | 5.2 | |
| Q99% | | 0.04 | 5.2 | 0.5 | 0.03 | 0.06 | 4.6 | 1.3 | 0.10 | 23 | 0.02 | 0.8 | |
| Min | | 1.19 | 26.2 | 0.7 | 1.39 | 1.10 | 28.6 | 1.9 | 1.55 | 176 | 1.10 | 2.7 | |
| Max | | 1.21 | 28.0 | 0.8 | 1.40 | 1.11 | 30.2 | 2.4 | 1.58 | 184 | 1.10 | 3.0 | |
| USP | [2013] | | | - | | | | <5 | | - | - | - | |

| | | | | | | | | | | | | | |
|---|---|---|---|---|---|---|---|---|---|---|---|---|---|
| TRASH | Rep | Total Trash Count | | Total Trash Size | | Dust Count | | Dust Mean Size | Trash Count | | Trash Mean Size | | VFM |
| | | [Cnt/g] | | [µm] | | [Cnt/g] | | [µm] | [Cnt/g] | | [µm] | | [%] |
| | 1 | 395 | | 66 | | 395 | | 66 | 0 | | 0 | | 0.03 |
| | 2 | 273 | | 70 | | 273 | | 70 | 0 | | 0 | | 0.02 |
| | 3 | 307 | | 67 | | 307 | | 67 | 0 | | 0 | | 0.02 |
| ⁿ | 3 | | | | | | | | | | | | |
| Mean | | 325 | | 68 | | 325 | | 68 | 0 | | 0 | | 0.02 |
| Std. Dev. | | 63 | | 2 | | 63 | | 2 | 0 | | 0 | | 0.00 |
| CV% | | 19.4 | | 3.1 | | 19.4 | | 3.1 | 0.0 | | 0.0 | | 10.0 |
| Q99% | | 361 | | 11 | | 351 | | 11 | 0 | | 0 | | 0.01 |
| Min | | 273 | | 66 | | 273 | | 66 | 0 | | 0 | | 0.02 |
| Max | | 395 | | 70 | | 395 | | 70 | 0 | | 0 | | 0.03 |
| USP | | | | | | | | | >95 | | <5 | | <5 |
| | [2013] | | | | | | | | | | | | |

**Table 3 Figures 4-7**

| NEP | Rep | Total Nep Cnt | | Total Nep Mean Size | | Fiber Nep Cnt | | FibNep Mean Size | | SCNep Count | | SCNep Mean Size | |
|---|---|---|---|---|---|---|---|---|---|---|---|---|---|
| | | [Cnt/g] | | [µm] | | [Cnt/g] | | [µm] | | [Cnt/g] | | [µm] | |
| | 1 | 11 | | 505 | | 11 | | 505 | | 0 | | 0 | |
| | 2 | 16 | | 525 | | 16 | | 525 | | 0 | | 0 | |
| | 3 | 2 | | 475 | | 2 | | 475 | | 0 | | 0 | |
| ⁿ | 3 | | | | | | | | | | | | |
| Mean | | 10 | | 502 | | 10 | | 502 | | 0 | | 0 | |
| Std. Dev. | | 7 | | 25 | | 7 | | 25 | | 0 | | 0 | |
| CV% | | 73.4 | | 5.0 | | 73.4 | | 5.0 | | 0.0 | | 0.0 | |
| Q99% | | 40 | | 143 | | 40 | | 143 | | 0 | | 0 | |
| Min | | 2 | | 475 | | 2 | | 475 | | 0 | | 0 | |
| Max | | 16 | | 525 | | 16 | | 525 | | 0 | | 0 | |
| USP | [2013] | <5 | | | | | | | | <5 | | | |

| | | | | | | | | | | | | | |
|---|---|---|---|---|---|---|---|---|---|---|---|---|---|
| LEN | Rep | L(w) | L(w) CV% | SFC(w) | UQL(w) | L(n) | L(n) CV% | SFC(n) | 5% L(n) | Fineness | Maturity Ratio | | IFC |
| | | [in] | [%CV] | %<0.5 in | [in] | [in] | [%CV] | %<0.5 in | [in] | [mtex] | [mat1] | | [%] |
| | 1 | 1.18 | 27.8 | 0.6 | 1.39 | 1.09 | 29.7 | 2.0 | 1.57 | 176 | 1.10 | | 2.8 |
| | 2 | 1.20 | 27.2 | 0.5 | 1.40 | 1.10 | 28.7 | 1.4 | 1.56 | 180 | 1.11 | | 2.4 |
| | 3 | 1.20 | 28.0 | 0.8 | 1.41 | 1.11 | 29.9 | 2.2 | 1.58 | 177 | 1.09 | | 3.3 |
| ⁿ | 3 | | | | | | | | | | | | |
| Mean | | 1.19 | 27.6 | 0.6 | 1.40 | 1.10 | 29.4 | 1.9 | 1.57 | 178 | 1.10 | | 2.8 |
| Std. Dev. | | 0.01 | 0.4 | 0.1 | 0.01 | 0.01 | 0.6 | 0.4 | 0.01 | 2 | 0.01 | | 0.4 |
| CV% | | 0.9 | 1.6 | 19.6 | 0.7 | 1.0 | 2.1 | 21.1 | 0.7 | 1.2 | 1.0 | | 15.7 |
| Q99% | | 0.06 | 2.5 | 0.7 | 0.05 | 0.06 | 3.6 | 2.3 | 0.07 | 11 | 0.06 | | 2.6 |
| Min | | 1.18 | 27.2 | 0.5 | 1.39 | 1.09 | 28.7 | 1.4 | 1.56 | 176 | 1.09 | | 2.4 |
| Max | | 1.20 | 28.0 | 0.8 | 1.41 | 1.11 | 29.9 | 2.2 | 1.58 | 180 | 1.11 | | 3.3 |
| USP | [2013] | | | - | | | | <5 | | - | - | | |

| | | | | | | | | | | | | | |
|---|---|---|---|---|---|---|---|---|---|---|---|---|---|
| Goes with Figures 4-7 | | | | | | | | | | | | | |

Some of the data in Tables 2 and 3 is illustrated as the histograms in Figures 27. Figures 2-4 correspond to Table 2 and Figures 5-7 correspond to Table 3.

Figure 2 is a histogram of fiber lengths by percent combined with a plot of fiber length versus cumulative percent, both factors being expressed by weight. As the tally columns further indicate, less than 13% (expressed as two significant figures) of the blend have lengths greater than 1.5 inches (3.81 cm) and only about 2.5% have lengths less than 0.75 inch (1.905 cm).

Figure 3 is a second histogram and plot based on the same sample with almost identical results: less than 14% are more than 1.5 inches (3.81 cm) in length and only about 5.6% are less than 0.75 inch (1.905 cm) in length.

Figure 4 is a fineness histogram based on the same sample as Figures 2 and 3 and the selected blend of deniers (1, 1.2, 1.5), expressed as mtex (i.e., 111, 133, and 167; all expressed to three significant figures). Figure 4 illustrates that 80% of the fibers (expressed to two significant figures) are between 250 and 100 mtex inclusive, and that 67% (2/3) are between 225 and 125 mtex inclusive.

Figure 5 is a histogram of fiber lengths by percent combined with a plot of fiber length versus cumulative percent for a second sample according to the invention, both factors being expressed by weight. As the Figure 5 tally columns further indicate, 8.0% (expressed as two significant figures) of the blend have lengths greater than 1.5 inches (3.81 cm) and only about 4.8% have lengths less than 0.75 inch (1.905 cm).

Figure 6 is a second histogram and plot based on the same sample with almost identical results: less than 12% are more than 1.5 inches (3.81 cm) in length and only about 4.0% are less than 0.75 inch (1.905 cm) in length.

Figure 7 is a fineness histogram based on the same second sample as Figures 5 and 6 and the selected blend of deniers (1, 1.2, 1.5), expressed as mtex (i.e., 111, 133, and 167; all expressed to three significant figures). Figure 7 illustrates that 81% of the fibers (expressed to two significant figures) are between 250 and 100 mtex inclusive, and that 68% (slightly more than 2/3) are between 225 and 125 mtex inclusive.

### Method

In another aspect the invention is a method of forming a yarn precursor blend with selected properties of moisture management and hand. In this aspect, the invention includes the steps of spinning continuous synthetic filament intodeniers and at least two different cross sections, gathering the different continuous filaments into a single tow, using a common cutter to cut the tow into staple lengths, and blending the different length, different denier and different cross-sectional staple fibers into an intimately blended bale. In particular, the method includes spinning the continuous synthetic filament into staple deniers (tex, fineness) of 1.0 dpf (111 mtex), 1.2 dpf (133 mtex) and 1.5 dpf (167 mtex); and using the common cutter to cut the tow into staple lengths of 1.5 inches (3.81 cm), 1.25 inches (3.175 cm), 1.0 inch (2.54 cm) and 0.75 inch (1.905 cm).

The filament (and then the fiber) cross sections are circular and oval. The oval (or elliptical) cross section offers increased surface area relative to an otherwise similarly sized round filament or fiber, and thus provides an additional design factor for moisture management.

The common cutter allows feeding and opening from one bale as opposed to drawing from multiple bales, each of which would have one of the separate characteristics. As known to those of skill in the art, the sooner different fibers are blended (i.e., earlier in the spinning process; baling, opening, drafting, etc.), the more consistent will be the characteristics for which the yarn was blended.

Thus, in another aspect, the invention is an intimately blended bale of polyester staple fibers that includes the combination of staple fibers with staple lengths of 1.5 inches (3.81 cm), 1.25 inches (3.175 cm), 1.0 inch (2.54 cm) and0.75 inch (1.905 cm); the combination of staple fibers with staple deniers (tex, fineness) of 1.0 dpf (111 mtex), 1.2 dpf (133 mtex) and 1.5 dpf (167 mtex); and the combination of staple fibers with at least two different staple cross sections including circular and oval cross sections. It follows that an opened bale of this type, and a yarn spun from this bale share the length, denier and cross-sectional characteristics of the intimately blended bale.

The intimately blended bale allows adjustment within a single bale and avoids the necessity to carefully meter fibers from multiple bales of different characteristics. The result is a yarn, and thus resulting fabrics, that are more consistent and precise on a weight for weight basis, and likewise avoid some of the more cumbersome aspects of other blending methods.

Therefore, in another aspect, the invention is a fabric that includes at least some yarns that consist essentially of: (1) a combination of polyester staple fibers with staple lengths of 1.5 inches (3.81 cm), 1.25 inches (3.175 cm), 1.0 inch (2.54 cm) and 0.75 inch (1.905 cm); (2) a combination of polyester staple fibers with staple deniers (tex, fineness) of 1.0 dpf (111 mtex), 1.2 dpf (133 mtex) and 1.5 dpf (167 mtex); and (3) a combination of polyester staple fibers with at least two different staple cross sections including circular and oval cross sections.

Such a fabric can be selected from the group consisting of woven fabrics, nonwoven fabrics, and knitted fabrics. Exemplary fabric embodiments include a blend of polyester fibers in the amounts of 20% by weight staple length of 1.5 inches (3.81 cm) or greater; 54% by weight staple lengths of 1.25 inches (3.175 cm) or greater; 77% by weight staple lengths of 1 inch (2.54 cm) or greater; and 96% by weight staple lengths of 0.75 inch (1.905 cm) or greater; with all lengths and percentages expressed to 2 significant figures.

Such exemplary fabrics can also be described as including 94% by weight of fibers at least 100 mtex; 87% by weight of fibers of at least 125 mtex; 76% by weight of fibers having at least 150 mtex: and 63% of fibers having at least 175 mtex; with all percentages expressed to 2 significant figures.

Also disclosed is a method of making a yarn with selected properties of moisture management and hand. The method includes the steps of opening an intimately blended bale of staple fibers in at least three different deniers, at least four different lengths, and at least two different cross sections, and forming the opened staple fibers into tow; forming the toe into a roving; and spinning the roving into yarn.

The intimately blended bale includes a combination of polyester staple fibers with staple lengths of 1.5 inches (3.81 cm), 1.25 inches (3.175 cm), 1.0 inch (2.54 cm) and 0.75 inch (1.905 cm); a combination of polyester staple fibers with staple deniers of 1.0 dpf (111 mtex), 1.2 dpf (133 mtex) and 1.5 dpf (167 mtex); a combination of polyester staple fibers with at least two different staple cross sections; 20% by weight staple length of 1.5 inches (3.81 cm) or greater; 54% by weight staple lengths of 1.25 inches (3.175 cm) or greater; 77% by weight staple lengths of 1 inch (2.54 cm) or greater; and 96% by weight staple lengths of 0.75 inch (1.905 cm) or greater; with all deniers, lengths and percentages expressed to 2 significant figures.

The method can include opening a bale that includes 94% by weight of fibers at least 100 mtex; 87% by weight of fibers of at least 125 mtex; 76% by weight of fibers having at least 150 mtex: and 63% of fibers having at least 175 mtex; with all percentages expressed to 2 significant figures.

A combination wire is typically used for carding a mixture of synthetic and natural fibers. Because the fiber blends according to the invention have a variable cut length that replicates the cumulative fiber length distribution curve of the pima cotton fibers as tested on the Uster AFIS (Advance Fiber Information System), a card with a combination wire was used to produce a 75 grain/yard sliver.

When fibers are only extended slightly in drafting there is a tendency for the high fiber-to-fiber cohesiveness to cause the fibers to snap back. To produce a yarn with better evenness values and fewer objectionable thin and thick places, the synthetic fibers should be extended far enough past each other to reduce fiber to fiber cohesion to a level that eliminates the snap back tendency.

When processing 100% cotton fibers the drawing creel weights are typically higher (500 grains or higher) and the drawing drafts are usually low (5.0 to 5.5) based upon the low fiber to fiber cohesion of cotton. Nevertheless, a high creel grain weight using synthetic fibers may create too much bulk between the steel roll and the top cot, limiting the amount of fiber control and degrade quality.

To manage the fiber to fiber cohesion, a two-step drawing process was utilized to combine different slivers creating a more homogeneous blending of the fibers. At the same time, a medium high draft (6.3 to 6.9) was utilized to extend the individual fibers further past each other which reduced the cohesiveness between the fibers.

By selecting a finer 1.3 HR (hank roving), the draft in roving was moved upward toward the mid-to-high range (9.67), which further extended the fibers past each other and further controlled the fiber to fiber cohesion.

The finer 1.3 HR reduced the ring spinning draft, which in turn allowed the ring frame drafting rolls to gain better control of the fibers. When spinning synthetic fibers it is important to manage roll chatter that is created by high fiber to fiber cohesion and an improper total draft and draft distribution. A high break draft (1.4 to 1.53) caused a slip-stick drafting of the fibers. The lower break draft (1.20) eliminated the chatter effect and produced better yarn evenness with fewer imperfections.

In all drafting processes, breaker drawing, finisher drawing, roving and, spinning, the roll space settings were adjusted based on the longest 5% length as measured on the Uster AFIS (Advance Fiber Information System) to prevent unwanted fiber damage and at the same time to further extend the longest fibers by removing hooks that were formed in carding. Each process was also evaluated on the Uster Evennes' tester (i.e., CV). The roll space and break drafts were adjusted to achieve a mass diagram without thick or thin places and a spectrogram without build ups (indicating fiber floating) or mechanical faults. Table 4 lists the settings in each process.

**Table 4**

| Carding: | Breaker Drawing | Finisher Drawing: | Roving: | Spinning: |
|---|---|---|---|---|
| Combination Wire | 450 grain Creel Wt. | 390 grain Creel Wt. | 68 mm M-B | 40/1 |
| | | | 1.3 Hank | 30.76 Total Draft |
| 75 gr/yd delivered | 44-53 mm roll settings | 44-53 mm roll settings | 1.104 Break Draft | |
| | | | | 70 mm M-B |
| | 1.40 Break Draft | 1.28 Break Draft | 9.67 Total Draft | 1.20 Break Draft |
| | 6.62 Total Draft | 6.3 Total Draft | | |
| | 65 grains/yard | 62 grains/yard | | 3.58 TM Yellow |
| | | | | |
| | | | | Distance Clips |

Other descriptions of the overall process in bringing staple to finished yarn can be found in Tortora, *supra*; or from Reiter Corporation (www.reiter.com/en/rikipedia) or from Cotton Incorporated (www.cottoninc.com).

Also disclosed is a cutter reel comprising blades spaced in positions that cut the fibers to the desired combination of lengths on a single reel.

Figure 8 illustrates a cutter reel assembled 10, and exploded 11. The cutter reel includes a top split cover 12, a bottom split cover 13, and a blade retainer 14. A top pin holder 15 and a bottom pin holder 16 together support a plurality of blade support pins 17. Slots 20 on the blade support pins 17 support the blades 21 for cutting the tow as the cutter reel rotates. The rotation is driven using the drive hub 22 in a manner well understood by those of ordinary skill in this art.

As illustrated, the cutter reel is based on US Patent No. 4497231.

In the drawings and specification there has been set forth a preferred embodiment of the invention, and although specific terms have been employed, they are used in a generic and descriptive sense only and not for purposes of limitation, the scope of the invention being defined in the claims.

## Claims

1. A spun yarn consisting essentially of a blend of polyester staple fibers customized by the parameter:
(1) a combination of polyester staple fibers with staple lengths of 1.5 inches (3.81 cm), 1.25 inches (3.175 cm), 1.0 inch (2.54 cm) and 0.75 inch (1.905 cm); **characterized by** the parameters:
(2) a combination of polyester staple fibers with staple deniers of 1.0 dpf (111 mtex), 1.2 dpf (133 mtex), and 1.5 dpf (167 mtex); and
(3) a combination of polyester staple fibers with at least two different staple cross sections that includes some staple fibers with circular cross sections and some with oval cross sections.

2. The yarn of Claim 1 comprising a blend of polyester fibers in the amounts of
20% by weight staple length of 1.5 inches (3.81 cm) or greater;
54% by weight staple lengths of 1.25 inches (3.175 cm) or greater;
77% by weight staple lengths of 1 inch (2.54 cm) or greater; and
96% by weight staple lengths of 0.75 inch (1.905 cm) or greater;
with all lengths and percentages expressed to 2 significant figures.

3. The yarn of Claim 1 comprising a blend of polyester fibers that includes:
94% by weight of fibers at least 100 mtex;
87% by weight of fibers of at least 125 mtex;
76% by weight of fibers having at least 150 mtex: and
63% of fibers having at least 175 mtex;
with all percentages expressed to 2 significant figures.

4. An intimately blended bale of polyester staple fibers comprising:
(1) a combination of staple fibers with staple lengths of 1.5 inches (3.81 cm), 1.25 inches (3.175 cm), 1.0 inch (2.54 cm) and 0.75 (1.905 cm) inch;
**characterized by**:
(2) a combination of staple fibers with staple deniers (tex, fineness) of 1.0 dpf (111 mtex), 1.2 dpf (133 mtex) and 1.5 dpf (167 mtex); and
(3) a combination of staple fibers with at least two different staple cross sections that includes some staple fibers with circular cross sections and some with oval cross sections.

5. A fabric that includes at least some yarns according to Claim 1.

6. The fabric according to Claim 5 selected from the group consisting of woven fabrics, nonwoven fabrics, and knitted fabrics.

7. The fabric according to Claim 5 comprising a blend of polyester fibers in the amounts of:
20% by weight staple length of 1.5 inches (3.81 cm) or greater;
54% by weight staple lengths of 1.25 inches (3.175 cm) or greater;
77% by weight staple lengths of 1 inch (2.54 cm) or greater; and
96% by weight staple lengths of 0.75 inch (1.905 cm) or greater;
with all lengths and percentages expressed to 2 significant figures.

8. The fabric according to Claim 5 comprising a blend of polyester fibers that includes:
94% by weight of fibers at least 100 mtex;
87% by weight of fibers of at least 125 mtex;
76% by weight of fibers having at least 150 mtex: and
63% of fibers having at least 175 mtex;
with all percentages expressed to 2 significant figures.

9. A method of making a yarn precursor blend with selected properties of moisture management and hand, the method comprising:
spinning continuous synthetic filament into deniers of 1.0 dpf (111 mtex), 1.2 dpf (133 mtex) and 1.5 dpf (167 mtex); and at least two different cross sections including circular and oval cross sections;
gathering the different continuous filaments into a single tow;
using a common cutter to cut the tow into staple lengths of 1.5 inches (3.81 cm), 1.25 inches (3.175 cm), 1.0 inch (2.54 cm) and 0.75 inch (1.905 cm); and
blending the different length, different denier and different cross-sectional staple fibers into an intimately blended bale.

10. The method according to Claim 9, wherein the intimately blended bale comprises a blend of polyester fibers in the amounts of:
20% by weight staple length of 1.5 inches (3.81 cm) or greater;
54% by weight staple lengths of 1.25 inches (3.175 cm) or greater;
77% by weight staple lengths of 1 inch (2.54 cm) or greater; and
96% by weight staple lengths of 0.75 inch (1.905 cm) or greater;
with all lengths and percentages expressed to 2 significant figures.

11. The method according to Claim 9, wherein the bale comprises a blend of polyester fibers that includes:
94% by weight of fibers at least 100 mtex;
87% by weight of fibers of at least 125 mtex;
76% by weight of fibers having at least 150 mtex: and
63% of fibers having at least 175 mtex;
with all percentages expressed to 2 significant figures.

## Patentansprüche

1. Ein gesponnenes Garn, das im Wesentlichen aus einer Mischung von Polyester-Stapelfasern besteht, und zwar angepasst an die folgenden Parameter:
(1) eine Kombination aus Polyester-Stapelfasern mit Stapellängen von 1,5 Zoll (3,81 cm), 1,25 Zoll (3,175 cm), 1,0 Zoll (2,54 cm) und 0,75 Zoll (1,905 cm);
**gekennzeichnet durch** die folgenden Parameter:
(2) eine Kombination aus Polyester-Stapelfasern mit Stapelfaser-Denier-Werten von 1,0 dpt (111 mtex), 1,2 dpt (133 mtex) und 1,5 dpt (167 mtex); und
(3) eine Kombination aus Polyester-Stapelfasern mit mindestens zwei verschiedenen Stapelfaserquerschnitten, die einige Stapelfasern mit kreisförmigen Querschnitten und einige mit ovalen Querschnitten aufweist.

2. Das Garn nach Anspruch 1, aufweisend eine Mischung aus Polyesterfasern in den folgenden Mengen:
20 Gew.-% Stapellängen von 1,5 Zoll (3,81 cm) oder mehr;
54 Gew.-% Stapellängen von 1,25 Zoll (3,175 cm) oder mehr;
77 Gew.-% Stapelfaserlängen von 1 Zoll (2,54 cm) oder mehr; und
96 Gew.-% Stapelfaserlängen von 0,75 Zoll (1,905 cm) oder mehr;
wobei alle Längen und Prozentsätze auf zwei geltende Ziffern angegeben sind.

3. Das Garn nach Anspruch 1, aufweisend eine Mischung aus Polyesterfasern, die Folgendes beinhaltet:
94 Gewichtsprozent Fasern mit mindestens 100 mtex;
87 Gewichtsprozent Fasern mit mindestens 125 mtex;
76 Gewichtsprozent Fasern mit mindestens 150 mtex; und
63 Gewichtsprozent Fasern mit mindestens 175 mtex;
wobei alle Prozentsätze auf zwei geltende Ziffern angegeben sind.

4. Ein eng verwobener Ballen aus Polyester-Stapelfasern, aufweisend:
(1) eine Kombination aus Stapelfasern mit Stapellängen von 1,5 Zoll (3,81 cm), 1,25 Zoll (3,175 cm), 1,0 Zoll (2,54 cm) und 0,75 Zoll (1,905 cm);
**gekennzeichnet durch**:
(2) eine Kombination aus Stapelfasern mit Stapel-Denier-Werten (Tex, Feinheit) von 1,0 dpt (111 mtex), 1,2 dpt (133 mtex) und 1,5 dpt (167 mtex); und
(3) einer Kombination aus Stapelfasern mit mindestens zwei verschiedenen Stapelquerschnitten, die einige Stapelfasern mit kreisförmigen Querschnitten und einige mit ovalen Querschnitten aufweist.

5. Ein Gewebe, das mindestens einige Garne gemäß Anspruch 1 enthält.

6. Das Gewebe gemäß Anspruch 5, ausgewählt aus der Gruppe bestehend aus gewebten Geweben, nicht gewebten Geweben und gestrickten Geweben.

7. Das Gewebe gemäß Anspruch 5, aufweisend eine Mischung aus Polyesterfasern in den folgenden Mengen:
20 Gew.-% Stapellängen von 1,5 Zoll (3,81 cm) oder mehr;
54 Gew.-% Stapellängen von 1,25 Zoll (3,175 cm) oder mehr;
77 Gew.-% Stapelfaserlängen von 1 Zoll (2,54 cm) oder mehr; und
96 Gew.-% Stapelfaserlängen von 0,75 Zoll (1,905 cm) oder mehr; wobei alle Längen und Prozentsätze auf zwei geltende Ziffern angegeben sind.

8. Das Gewebe gemäß Anspruch 5, aufweisend eine Mischung aus Polyesterfasern, die Folgendes beinhaltet:
94 Gewichtsprozent Fasern mit mindestens 100 mtex;
87 Gewichtsprozent Fasern mit mindestens 125 mtex;
76 Gewichtsprozent Fasern mit mindestens 150 mtex; und
63 Gewichtsprozent Fasern mit mindestens 175 mtex;
wobei alle Prozentsätze auf zwei geltende Ziffern angegeben sind.

9. Ein Verfahren zur Herstellung einer Garnvorläufermischung mit ausgewählten Eigenschaften hinsichtlich Feuchtigkeitsmanagement und Griff, wobei das Verfahren Folgendes aufweist:
Spinnen von kontinuierlichen synthetischen Filamenten zu Denier-Werten von 1,0 dpt (111 mtex), 1,2 dpt (133 mtex) und 1,5 dpt (167 mtex); und mindestens zwei unterschiedlichen Querschnitte, einschließlich kreisförmiger und ovaler Querschnitte;
Sammeln der verschiedenen Endlosfilamente zu einem einzigen Werg;
Verwenden eines gemeinsamen Schneidwerkzeugs zum Schneiden des Wergs in Stapellängen von 1,5 Zoll (3,81 cm), 1,25 Zoll (3,175 cm), 1,0 Zoll (2,54 cm) und 0,75 Zoll (1,905 cm); und
Mischen der Stapelfasern unterschiedlicher Länge, unterschiedlicher Denier-Werte und unterschiedlicher Querschnitte zu einem eng verwobenen Ballen.

10. Das Verfahren nach Anspruch 9, wobei der eng verwobener Ballen eine Mischung aus Polyesterfasern in den folgenden Mengen aufweist:
20 Gew.-% Stapellängen von 1,5 Zoll (3,81 cm) oder mehr;
54 Gew.-% Stapellängen von 1,25 Zoll (3,175 cm) oder mehr;
77 Gew.-% Stapelfaserlängen von 1 Zoll (2,54 cm) oder mehr; und
96 Gew.-% Stapelfaserlängen von 0,75 Zoll (1,905 cm) oder mehr;
wobei alle Längen und Prozentsätze auf zwei geltende Ziffern angegeben sind.

11. Das Verfahren nach Anspruch 9, wobei der Ballen eine Mischung aus Polyesterfasern aufweist, die Folgendes enthält:
94 Gewichtsprozent Fasern mit mindestens 100 mtex;
87 Gewichtsprozent Fasern mit mindestens 125 mtex;
76 Gewichtsprozent Fasern mit mindestens 150 mtex; und
63 Gewichtsprozent Fasern mit mindestens 175 mtex;
wobei alle Prozentsätze auf zwei geltende Ziffern angegeben sind.

## Revendications

1. Filé de fibres constitué essentiellement d'un mélange de fibres courtes de polyester et personnalisé par le paramètre suivant :
(1) une combinaison de fibres courtes de polyester présentant des longueurs de fibre de 1,5 pouces (3,81 cm), 1,25 pouces (3,175 cm), 1,0 pouce (2,54 cm) et 0,75 pouce (1,905 cm) ;
**caractérisé par** les paramètres suivants :
(2) une combinaison de fibres courtes de polyester présentant des deniers de base de 1,0 dpf (111 mtex), 1,2 dpf (133 mtex) et 1,5 dpf (167 mtex) ; et
(3) une combinaison de fibres courtes de polyester présentant au moins deux sections de fibre courtes différentes incluant des fibres de section circulaire et certaines de section ovale.

2. Filé de fibres selon la revendication 1, comprenant un mélange de fibres de polyester dans les quantités de
20 % en poids de fibres courtes d'une longueur de 1,5 pouces (3,81cm) ou plus ;
54 % en poids de fibres courtes d'une longueur de 1,25 pouces (3,175 cm) ou plus ;
77 % en poids de fibres courtes d'une longueur de 1 pouce (2,54 cm) ou plus ; et
96 % en poids de fibres courtes d'une longueur de 0,75 pouce (1,905 cm) ou plus ;
toutes les longueurs et pourcentages étant exprimés selon une précision à deux chiffres significatifs.

3. Filé de fibres selon la revendication 1, comprenant un mélange de fibres incluant :
94 % en poids de fibres d'au moins 100 mtex ;
87 % en poids de fibres d'au moins 125 mtex ;
76 % en poids de fibres d'au moins 150 mtex ; et
63 % de fibres d'au moins 175 mtex ;
tous les pourcentages étant exprimés selon une précision à deux chiffres significatifs.

4. Balle intimement mélangée de fibres courtes de polyester comprenant :
(1) une combinaison de fibres courtes présentant des longueurs de fibre de 1,5 pouces (3,81 cm), 1,25 pouces (3,175 cm), 1,0 pouce (2,54 cm) et 0,75 pouce (1,905 cm) ;
**caractérisé par** :
(2) une combinaison de fibres courtes présentant des deniers de fibres (tex, finesse) de 1,0 dpf (111 mtex), 1,2 dpf (133 mtex) et 1,5 dpf (167 mtex) ; et
(3) une combinaison de fibres courtes présentant au moins deux sections de fibre différentes et incluant des fibres de section circulaire et certaines de section ovale.

5. Tissu incluant au moins quelques fibres selon la revendication 1.

6. Tissu selon la revendication 5 sélectionné dans le groupe constitué de tissus tissés, de tissus non tissés et de tricots.

7. Tissu selon la revendication 5 comprenant un mélange de fibres de polyester dans les quantités de :
20 % en poids de fibres discontinues d'une longueur de 1,5 pouce (3,81 cm) ou plus ;
54 % en poids de fibres courtes d'une longueur de 1,25 pouces (3,175 cm) ou plus ;
77 % en poids de fibres courtes d'une longueur de 1 pouce (2,54 cm) ou plus ; et
96 % en poids de fibres courtes d'une longueur de 0,75 pouce (1,905 cm) ou plus ;
toutes les longueurs et pourcentages étant exprimés selon une précision à deux chiffres significatifs.

8. Tissu selon la revendication 5 comprenant un mélange de fibres de polyester incluant :
94 % en poids de fibres d'au moins 100 mtex ;
87 % en poids de fibres d'au moins 125 mtex ;
76 % en poids de fibres d'au moins 150 mtex ; et
63 % de fibres d'au moins 175 mtex ;
tous les pourcentages étant exprimés selon une précision à deux chiffres significatifs.

9. Procédé de fabrication d'un mélange précurseur de fil présentant des propriétés sélectionnées de gestion de l'humidité et de toucher, le procédé comprenant les étapes suivantes :
filer un filament synthétique continu en deniers de 1,0 dpf (111 mtex), 1,2 dpf (133 mtex) et 1,5 dpf (167 mtex) et au moins deux sections différentes incluant des sections circulaire et ovale ;
rassembler les différents filaments continus en une étoupe ;
utiliser un dispositif de coupe pour découper l'étoupe en longueurs de fibre discontinue de 1,5 pouces (3,81 cm), 1,25 pouces (3,175 cm), 1,0 pouce (2,54 cm) et 0,75 pouce (1,905 cm) ; et
mélanger les fibres courtes de différentes longueurs, différents deniers et différentes sections en une balle intimement mélangée.

10. Procédé selon la revendication 9, dans lequel la balle intimement mélangée comprend un mélange de fibres de polyester dans les quantités de :
20 % en poids de fibres courtes d'une longueur de 1,5 pouces (3,81 cm) ou plus ;
54 % en poids de fibres courtes d'une longueur de 1,25 pouces (3,175 cm) ou plus ;
77 % en poids de fibres courtes d'une longueur de 1 pouce (2,54 cm) ou plus ; et
96 % en poids de fibres courtes d'une longueur de 0,75 pouce (1,905 cm) ou plus ;
toutes les longueurs et pourcentages étant exprimés selon une précision à deux chiffres significatifs.

11. Procédé selon la revendication 9, dans lequel la balle comprend un mélange de fibres de polyester incluant :
94 % en poids de fibres d'au moins 100 mtex ;
87 % en poids de fibres d'au moins 125 mtex ;
76 % en poids de fibres d'au moins 150 mtex ; et
63 % de fibres d'au moins 175 mtex ;
tous les pourcentages étant exprimés selon une précision à deux chiffres significatifs.
